

No. 890,231.

PATENTED JUNE 9, 1908.

J. T. JONES.  
METHOD OF TREATING ORE.  
APPLICATION FILED DEC. 23, 1907.



## Witnesses.

Edw. Gaylord.  
Chas. Bull.

Inventor:

John T. Jones,

Beaupre-en-Beth, *Co. Chittenden, Vt.*  
*At the same*

# UNITED STATES PATENT OFFICE.

JOHN T. JONES, OF IRON MOUNTAIN, MICHIGAN, ASSIGNOR OF ONE-HALF TO GEORGE A. ST. CLAIR, OF DULUTH, MINNESOTA.

## METHOD OF TREATING ORE.

No. 890,231.

Specification of Letters Patent.

Patented June 9, 1908.

Application filed December 23, 1907. Serial No. 407,770.

To all whom it may concern:

Be it known that I, JOHN T. JONES, a citizen of the United States, residing at Iron Mountain, in the county of Dickinson and State of Michigan, have invented a new and useful Improvement in Methods of Treating Ore, of which the following is a specification.

The object of my invention is to provide a novel method of treating, by furnace-operation, ore containing iron, zinc and sulfur as its principal constituents; and I have more especially devised my invention for the treatment of a certain ore containing about 31 per cent. iron, about 17 per cent. zinc, about 15 30 to 33 per cent. sulfur, and about 5 to 7 per cent. silica. The treatment consists, generally stated, in subjecting successively the ore to heat sufficient to burn out the sulfur but insufficient to volatilize the zinc, and the remainder of the ore to a higher degree of heat sufficient to volatilize the zinc, which is carried off and condensed, the remnant of the ore, containing iron and earthy material, coming down in the furnace-stack, under the action of the heat, in the form of matte, which may be disposed of in the manner hereinafter described.

The accompanying drawing shows, by a broken view in sectional elevation, a furnace-equipment suitable for the practice of my invention.

For carrying out my invention to the best advantage, a site should be selected on the side of a hill for the erection of two furnace-structures 1 and 2. The upper structure 1 consists of a carbonaceous-fuel-burning furnace 3, adapted to burn soft-coal, as the most suitable fuel, on a grate 4 in the furnace-chamber above an air-blast opening 5 in the chamber-wall, below which is indicated a conveyor 6 for carrying off the ashes. This fuel-furnace is supported on a suitable foundation 7 to extend parallel with an ore-stack 8 rising from a foundation 9 to a height of one hundred feet, more or less, and with the base-portion of which a flue-forming neck 10 communicates, leading thereto from a point about midway between the upper and lower ends of the fuel-chamber. By extending the flue from this point the gases from the lower portion of the fuel-bed, which is raised to and maintained at incandescence up to the plane of the neck, and the hydrocarbons distilled off from the upper portion of the fuel-bed by

the heat below it, are drawn through the flue 55 into the stack 8. This stack and the furnace 3 may be constructed of or lined with suitable brick, preferably of the magnesite variety, but the neck 10 is best made of carbonaceous material to adapt it to resist the destructive tendency of the heat from the gases mixing in and coursing through it, the material I prefer to employ for the purpose being blocks of graphite carbon, or a mixture of pulverized graphite and coke with a suitable 60 binder, as coal-tar, compacted by hydraulic pressure to solidify the mass and then baked to harden it.

From the open lower end of the ore-stack a chute 11, having a hinged valve 12 interposed in it, inclines downwardly to discharge into a hopper 13 surmounting the upper end of the relatively short ore-stack 14 of the structure 2, formed like the stack 8, and communicating from between its ends through a flue-forming neck 15, with the chamber of a fuel-furnace 16 of this last-named structure, this furnace being in all particulars, by preference, like and operating the same as the furnace 3. In the wall of the stack 14 opposite site that with which the flue 15 connects, and alining with the flue, is provided a discharge-opening 17 leading to a conduit 18, which inclines upwardly along the hill-side, at an angle of, say, about 45 degrees, and may be a 80 thousand feet, more or less, in length. This conduit, which contains normally closed openings 19 at suitable intervals apart throughout its length, may best be formed of a net-work of wire embedded in concrete and 85 molded in sections of cylindrical or other desired shape. The lower end of the ore-stack is open to an inclined chute 20 leading down the hill to any desired point to which it is desired to deliver the remnant of the 90 treated ore.

The procedure is as follows: With the fire burning in the furnace 3, and supplied with combustion-promoting air through a port 22, and the stack filled, to the closed valve 12, 100 with the ore to be treated, the hot gases passing through the flue 10 into the stack and upward therein through the interstitial column of ore, burn out the sulfur-constituent of the ore, the heat being regulated to an intensity 105 only sufficient to drive off the sulfur, and this sulfur-burning action being supplemented by the admission of air into the stack through a

port 21 near its base. From time to time, on opening the valve 12, the sulfur-free ore at the base of the stack is permitted to fall through the chute 11 to charge the stack 14 therewith. The hot ore in this stack is subjected to the action of the gases from the furnace 16, passing into the stack through the flue 15 at a temperature of from about twenty-two hundred to twenty-five hundred 10 degrees F., which is sufficient to volatilize the zinc-constituent of the ore, the fumes of which pass through the restricted outlet 17 into the conduit 18 and become condensed in their course through the latter dropping 15 therein in the form of flakes, the accumulations of which may be withdrawn from time to time through the openings 19. The remainder of the ore, containing iron and earthy material reduced by the heat to matte- 20 form, falls down the chute 20 to the point of delivery, whence it may be taken for use as a flux after treating it in known manner, if it contains gold, to recover the gold from it.

What I claim as new and desire to secure 25 by Letters Patent is—

1. The method of treating ore containing sulfur, zinc and iron, which consists in successively subjecting said ore to the action of hot fuel-gas at relatively lower and higher 30 temperature to first burn out the sulfur and

then volatilize the zinc, and recovering the zinc by condensation.

2. The method of treating ore containing sulfur, zinc and iron, which consists in first subjecting said ore to the action of gases 35 from carbonaceous fuel at a temperature sufficient to burn out the sulfur but insufficient to volatilize the zinc, then subjecting the sulfur-free ore to the action of similar gases at a higher temperature sufficient to 40 volatilize the zinc, and condensing the zinc-fumes, for the purpose set forth.

3. The method of treating ore containing sulfur, zinc and iron, which consists in first subjecting said ore to the action of gases 45 from carbonaceous fuel at a temperature sufficient to burn out the sulfur but insufficient to volatilize the zinc, and introducing air into the ore to enhance the burning of the sulfur, then subjecting the sulfur-free ore 50 to the action of similar gases at a higher temperature sufficient to volatilize the zinc but insufficient to melt the iron, condensing the zinc-fumes to recover the zinc, and saving the iron-containing remnant of the ore.

JOHN T. JONES.

In presence of:—

K. M. CORNWALL,  
R. A. SCHAEFER.